# EUROPEAN PATENT SPECIFICATION

(11) **EP 0 172 955 B1**
(45) Date of publication and mention of the grant of the patent: **08.02.1989**
(21) Application number: 84305857.9
(22) Date of filing: 28.08.1984
(51) Int. Cl.: D01F 9/14

(54) **A method for producing a precursor pitch for carbon fiber**
Verfahren zur Herstellung eines Vorläuferpechs für Kohlenstoffaser
Méthode pour la production d'un brai précurseur pour une fibre de carbone

(43) Date of publication of application: 05.03.1986
(73) Proprietor: KAWASAKI STEEL CORPORATION, Chuo-Ku, Kobe-City Hyogo 651 (JP)
(72) Inventor: Yudate, Kozo c/o Research Laboratories, Chiba City (JP); Nakasawa, Ken c/o Research Laboratories, Chiba City (JP)
(74) Representative: Overbury, Richard Douglas

(56) References cited:
- EP-A- 0 089 840
- DERWENT JAPANESE PATENTS REPORT, Derwent Publications, Section Chemical, vol. 6, no. 239 (C-137)[1117], 26th November 1982; & JP - A - 57 139 179 (KAWATETSU KAGAKU K.K.)

## Description

The present invention relates to a method for producing a precursor pitch for carbon fiber preparation and is concerned with a method wherein coal tar soft or middle pitch is subjected to heat-treatment to form mesophase pitch.

The production of carbon fibers is generally classified into methods using synthetic fibers such as polyacrylonitrile, etc. as the raw material and methods using a petroleum pitch or a coal tar pitch as the raw material. The former method has the drawbacks that the raw material fiber is expensive and the carbonization yield of the raw material fiber is low. In the latter method, there is the drawback that pitch having a good spinnability has poor infusibility whereas pitch having a good infusibility has poor spinnability. Presently commercially available carbon fibers are almost always formed using petroleum pitch as the raw material. But, when petroleum pitch is used as the raw material, it is essential to effect the removal of insoluble solid components to adjust the raw material pitch and a variety of specific physical chemical treatments such as hydrogenation, heat treatment and the like have to be carried out and these steps involve much labour and time.

When coal tar pitch is used as the raw material, it is necessary to separate and remove microparticles of free carbon having a diameter of less than 1 11m contained in the pitch as an insuluble solid component and in order to improve the spinnability and infusibility, specific adjustments of the pitch, such as by using a plurality of solvents, hydrogenation, heat treatment and the like, are carried out.

In general, the following properties are demanded for a precursor for carbon fiber:-
(1) No insoluble solid components, such as ash, free carbon, etc.
(2) Excellent heat stability
(3) High melt spinnability
(4) Easy infusible treatment.
(5) High carbonization yield.

Carbon fibers obtained by melt-spinning precursor pitch having such properties and subjecting the spun fiber to infusibilizing and carbonizing treatments have excellent graphitization and orientation and have the desired strength and Young's modulus properties.

The inventors have diligently studied to obtain a precursor pitch having the above described properties and have found a method for producing precursor pitch for carbon fiber which satisfactorily satisfies concurrently the above described requirements for precursor pitch for carbon fibers. In this method free carbon in the coal tar pitch can be easily removed and specific treatments such as hydrogenation and the like are not needed.

EP-A-008984 describes a process for the production of a pitch for use in the preparation of carbon fibers. In this process a suitable starting material is subjected to a first heat treatment to remove volatile matter and is then allowed to settle to form an upper layer and a lower layer. The lower layer is a pitch which is largely an optically anisotropic phase. The upper layer is again subjected to heat treatment to obtain an optically anistropic pitch which can be melt spun to form a carbon fibre. Suitable starting materials are carbonaceous heavy oils, tars and pitches obtained from the petroleum or coal industry.

According to the present invention there is provided a method of producing a pitch suitable for the preparation of carbon fibres which method comprises
(i) heating, in a first stage, a pitch obtained from the coal industry
(ii) extracting the thus heat treated pitch with a solvent,
(iii) separating and removing the solvent insoluble portion together with free carbon, and
(iv) heating, in a second stage, the solvent soluble portion characterised in that
(v) the pitch obtained from the coal industry is a soft or middle coal tar pitch having a softening point of 50 to 75°C,
(vi) the coal tar pitch is heated, in the first stage at a temperature of 350 to 500°C in an inert gas atmosphere to form mesophase,
(vii) the solvent is an aromatic solvent
(viii) the solvent insoluble portion includes the mesophase, and
(ix) the solvent soluble portion contains no free carbon and is heated, in the second stage, in an inert gas atmosphere under atmospheric pressure or a reduced pressure to form a bulk mesophase pitch containing 20-60% by weight if a quinoline insoluble portion.

For a better understanding of the invention and to show how the same may be carried into effect, reference will now be made, by way of example, to the accompanying drawing which shows a graph illustrating the relationship between the heat treatment temperature (T°C) in the production of the precursor pitches for carbon fibers and the time (0 min) for which said temperature is held.

According to the present invention, the coal tar pitch is heat-treated in the first stage to form mesophase. Then a solvent insoluble portion including the mesophase is separated and removed by extraction using an aromatic solvent, whereby free carbon contained in the pitch can be easily removed and pitch containing no free carbon is obtained. According to this method, it is possible to easily produce a precursor pitch for carbon fibers which has a very high thermal stability, excellent spinnability and infusibility, a high carbonization yield and excellent graphitization and orientation without needing specific treatments such as hydrogenation and the like as hitherto.

The formation of the mesophase, the growth thereof, and the assembling thereof when the pitch is heat-treated, are somewhat different depending upon the kind of pitch but the mesophase is formed from a temperature of about 350°C. When the temperature is further raised, the formed amount increases and the mesophase grows to form large globular bodies. From about 470°C, the mesophase assembles and at about 500°C, the mesophase is wholly formed into an anisotropic body. In the course of the reaction, the fine particles of free carbon having a diameter of less than 1 11m and inorganic substances which become ash, which ar originally present in the coal tar pitch, stick around the mesophase globular bodies and hence are easily removed with the mesophase.

Furthermore, high molecular weight components having a high thermal reactivity which are present in the pitch and components having a small content of functional groups are preferentially polycondensed to remove these substances and form the mesophase, so that the resulting pitch is low in the amount of heteroatoms and is homogeneous and has excellent thermal stability.

In the present invention, the pitch is heat-treated at a temperature from about 350°C at which the mesophase is formed to about 500°C at which the whole coke formation proceeds, in the first stage. When the temperature of the heat treatment is too high, the mesophase is formed in a large amount and as a result, the yield of hard pitch lowers. Conversely, when the temperature of the heat treatment is too low, the components having a high thermal reactivity are apt to remain in the hard pitch. When these two converse conditions are taken into account, the temperature of the heat treatment is optimum at about 350°C-500°C as mentioned above and it is preferable to form 10-30% by weight of the mesophase within this temperature range.

By adding an aromatic solvent to the pitch in which the mesophase has been formed by the heat treatment under these conditions, the solvent insoluble portion including the mesophase is easily separated through spontaneous precipitation or filtration. The separation of the mesophase by filtration does not cause clogging of the mesh of the filter, as tends to occur during the filtration of free carbon, and is very easy. Thereafter, the solvent is removed by distillation to obtain pitch having no free carbon. This pitch is heat-treated in the second stage to form mesophase, whereby the desired precursor pitch suitable for carbon fiber production is obtained. This precursor has a softening point higher than 300°C and consists of 80-95% by weight of a benzene insoluble portion, 20-60% by weight of a quinoline insoluble portion and less than 800 ppm of ash.

The precursor pitch for carbon fiber obtained according to the present invention is so-called "bulk mesophase pitch" containing 20-60% by weight of a quinoline insoluble portion. When this pitch is observed with a polarizing microscope, it can be seen that an isotropic pitch component is dispersed in the whole optical anistropic texture. The ratio of the optical anistropic texture observed under the polarizing microscope is 80-95%. It has been found that such a pitch has excellent spinnability and infusibility and can provide carbon fibers having high strength and Young's modulus. The carbon fibers formed from the mesophase pitch have various properties which have never been seen in carbon fibers made of isotropic precursor pitch containing no mesophase. That is, carbon fibers made from the mesophase pitch according to the present invention show high Young's modulus even at a treating temperature of 1,000°C and both the tensile strength and the Young's modulus are noticeably more improved by a graphitizing treatment.

The most suitable precursor pitch for carbon fiber is a mesophase pitch having 80-95% by weight of benzene insoluble portion and 20-60% by weight of quinoline insoluble portion. When the benzene insoluble portion is less than 80% by weight and the quinoline insoluble portion is less than 20% by weight, the mesophase portion and the isotropic pitch portion in the mesophase pitch separate and such a pitch cannot be spun. When the benzene insoluble portion is more than 95% by weight and the quinoline insoluble portion is more than 60% by weight, the melt viscosity of the mesophase pitch is quite high and spinning is not feasible. In mesophase pitch having 80-95% by weight of benzene insoluble portion and 20-60% by weight of quinoline insoluble portion, the mesophase portion and the isotropic pitch portion are present in a uniform system, the melt viscosity at the spinning temperature is not high, and the spinnability is excellent.

Thus, a mesophase pitch having a softening point of higher than 300°C, 80-95% by weight of benzene insoluble portion and 20-60% by weight of quinoline insoluble portion is suitable as a precursor pitch for carbon fiber. It has a uniform system, excellent thermal stability, spinnability and infusibility, and has a high carbonization yield and few impurities, such as free carbon, heteroatoms, and inorganic substances. Carbon fibers formed therefrom have high strength and Young's modulus.

The method for preparing the precursor for carbon fibers by heat-treating, in the second stage, the pitch containing no free carbon which has been obtained by the heat treatment in the first stage, is a simple one which comprises heating the pitch under atmospheric pressure or a reduced pressure in an inert gas atmosphere to form the mesophase pitch as mentioned above. The precursor pitch obtained has excellent thermal stability and is suitable for spinning, because the high molecular weight components having high thermal reactivity and heteroatoms present in the raw material pitch are removed by the heat treatment at the first stage. Furthermore, since the raw material for the pitch is coal tar pitch rich in aromatic materials and the heat treatment is applied at the first stage, the resulting pitch containing no free carbon is composed of relatively large aromatic molecules. Therefore, in the mesophase pitch obtained in the second stage, the mesophase component and the isotropic component are present in a uniform system.

The heat treatment of the pitch containing no free carbon in the second stage is intended to produce bulk mesophase pitch having 20-60% by weight of quinoline insoluble portion and 80-95% by weight of benzene insoluble portion and it has been found, from a large number of experiments, that the heat treatment temperature (T°C) and the time (8 min) for which this temperature should be held preferably have the following relationship:-

That is, if the heat treatment temperature (T°C) and the time (8 min) for holding this temperature satisfy the requirement of the above equation (1), a a bulk mesophase pitch having 20-60% by weight of quinoline insoluble portion and 80-95% by weight of benzene insoluble portion can be obtained. This bulk mesophase pitch becomes the precursor pitch for high performance carbon fibers (abbreviated as "HP carbon fibers" hereinafter) having high strength and high elasticity.

When the pitch containing no free carbon is heat-treated, a precursor pitch for general purpose carbon fiber (abbreviated as "GP carbon fiber" hereinafter) having low elasticity can be obtained but this pitch is an isotropic pitch and is different from the mesophase pitch. In this case, it has been found that the heat treatment temperature (T°C) and the time (θ min) at which this temperature should be held have the following relationship:-

The relations of the above equations (1) and (2) are shown in Fig. 1.

As can be seen from Fig. 1, when the bulk mesophase pitch which is the precursor pitch of HP carbon fiber is compared with the isotropic pitch which is the precursor pitch of GP carbon fiber, the heat treatment holding time of the former pitch is longer than that of the latter pitch.

Ash which is an impurity in the precursor pitch causes the formation of voids in carbon fibers or deteriorates the strength, so that the amount of the remaining free carbon is preferred to be as small as possible. However, the precursor pitch according to the present invention is very clean, as the ash content is less than 300 ppm, and is a very excellent carbon fiber precursor.

This precursor pitch is melt-spun at a temperature higher by 20―40°C than the softening point by means of the conventional melt-spinnning techniques.

The spun fibers may be subjected to an infusing treatment by air oxidation without effecting pretreatment or by using an oxidizing agent, such as ozone oxidation or sulfuric acid. After this infusing treatment, the spun fibers are fired and carbonized by raising the temperature up to about 1,000°C in an inert gas such as Ar, N₂ to obtain carbon fibers. By further firing and graphitizing the carbon fibers at a temperature of higher than 2,000°C, graphite fibers having high strength and Young's modulus can be obtained without carrying out a drawing step or the like.

The following Examples illustrate the invention.

### Example 1

Coal tar soft pitch having a softening point in the range 50 to 75°C and containing free carbon was heated at 450°C in an inert gas atmosphere for 60 minutes to form 25% by weight of mesophase and then the thus treated pitch was extracted with tar oil (an aromatic solvent). The high molecular weight components, which were mainly mesophase, were then filtered off. The filtrate was vacuum-distilled to recover the solvent and to obtain pitch having a softening point of 90°C, 12% by weight of benzene insoluble portion, and a trace of quinoline insoluble portion and containing no free carbon. This pitch was heat-treated at 465°C under a vacuum of 20 mmHg in N₂ inert gas atmosphere to obtain mesophase pitch having a softening point of 355°C, and consisting of 91.9% by weight of benzene insoluble portion and 55.2% by weight of quinoline insoluble portion. When this pitch was observed with a polarizing microscope, it was seen that an isotropic pitch component was dispersed in the optical anisotropic texture. The ratio of the optical anisotropic texture was 86%. This mesophase pitch was melt-spun at 385°C at a take-up rate of 300-500 m/min and the spun fiber was oxidized in air at 320°C and subsequently carbonized at 1,000°C in an argon atmosphere to obtain a carbon fiber. This fiber had a fineness of 12-14 µm. a tensile strength of 140 kg/mm² and Young's modulus of 8.4 t/mm². Furthermore, this fiber was graphitized at 2,600°C in argon atmosphere to obtain a graphite fiber. This fiber had a fineness of 11-13 um, a tensile strength of 240 kg/mm² and Young's modulus of 48 t/mm².

### Example 2

Samples of the pitch containing no free carbon obtained in the first heat treatment stage in Example 1 'were heated at 465°C under atmospheric pressure for 30, 60 and 180 minutes respectively. At this time, N₂ inert gas was introduced at a flow rate of 5 I/min based on 300 g of the pitch. The pitches heat treated for 30, 60 and 180 minutes are referred to as (I), (II) and (III) and the obtained results are shown in the following Table 1. In pitch (I), the mesophase portion and the isotropic pitch portion separated upon melt-spinning and spinning was not feasible. Pitch (III) had quite a high melt viscosity and was impossible to spin. Only mesophase pitch (II) could be melt-spun at 370°C at a take-up rate of 300-500 m/min. The spun fiber was oxidized in air at 320°C and then carbonized at 1,000°C in an argon atmosphere to obtain a carbon fiber. This fiber had a fineness of 12-14 pm, a tensile strength of 130 kg/mm² and Young's modulus of 8.6 t/mm². Furthermore, graphitization was effected at 2,600°C in an argon atmosphere to obtain a graphite fiber. This fiber had a fineness of 11-13 pm, a tensile strength of 280 kg/mm² and Young's modulus of 43 t/mm².

Comparative Example 1

Coal tar soft pitch containing free carbon was directly extracted with tar oil without effecting a heat treatment. A pitch having a softening point of 90°C and containing a trace of quinoline insoluble portion and still containing free carbon was obtained by filtration. This pitch was heat-treated at 450°C under a vacuum of 20 mmHg in N₂ gas atmosphere for 60 minutes to obtain mesophase pitch having 82.8% by weight of benzene insoluble portion and 43.2% by weight of quinoline insoluble portion. Phase separation between the mesophase portion and the isotropic pitch portion occurred in the molten state and it was impossible to carry out spinning.

## Claims

1. A method for producing a pitch suitable for the preparation of carbon fibres which method comprises.

(i) heating, in a first stage, a pitch obtained from the coal industry,
(ii) extracting the thus heat treated pitch with a solvent,
(iii) separating and removing the solvent insoluble portion together with free carbon, and
(iv) heating, in a second stage, the solvent soluble portion characterised in that
(v) the pitch obtained from the coal industry is a soft or middle coal tar pitch having a softening point of 50 to 75°C,
(vi) the coal tar pitch is heated, in the first stage, at a temperature of 350 to 500°C in an inert gas atmosphere to form mesophase,
(vii) the solvent is an aromatic solvent,
(viii) the solvent insoluble portion includes the mesophase, and
(ix) the solvent soluble portion contains no free carbon and is heated, in the second stage, in an inert gas atmosphere under atmospheric pressure or a reduced pressure to form a bulk mesophase pitch containing 20-60% by weight if a quinoline insoluble portion.

2. A method as claimed in claim 1, wherein the heat treatment of the solvent soluble portion in the second stage is effected under the following condition wherein T(°C) is the temperature of the heat treatment and 8 (min) is the time for which said portion is held at said temperature.

## Patentansprüche

1. Verfahren zur Erzeugung eines für die Herstellung von Kohlenstoffasern geeigneten Pechs, umfassend

(i) das Erhitzen, in einer ersten Stufe, eines von der Kohle-Industrie erhalten Pechs,
(ii) das Extrahieren des so wärmebehandelten Pechs mit einem Lösungsmittel,
(iii) das Abtrennen und Entfernen des in dem Lösungsmittel unlöslichen Anteils zusammen mit freiem Kohlenstoff, und
(iv) das Erhitzen, in einer zweiten Stufe, des in dem Lösungsmittel löslichen Anteils, dadurch gekennzeichnet, daß
(v) das von der Kohle-Industrie erhaltenen Pech ein Weichkohlen- oder Mittelkohlenteer-Pech mit einem Erweichungspunkt von 50°C bis 75°C ist,
(vi) das Kohlenteer-Pech in der ersten Stufe in einer Inertgas-Atmosphäre auf eine Temperatur von 350°C bis 500°C zur Bildung einer Mesophase erhitzt wird,
(vii) das Lösungsmittel, ein aromatisches Lösungsmittel ist,
(viii) der in dem Lösungsmittel unlösliche Anteil die Mesophase enthält und
(ix) der in dem Lösungsmittel lösliche Anteil keinen freien Kohlenstoff enthält und, in der zweiten Stufe, in einer Inertgas-Atmosphäre unter Atmosphären-Druck oder vermindertem Druck zur Bildung eines massiven Mesophasen-Pechs erhitzt wird, das 20 bis 60 Gew.-% eines in Chinolin unlöslichen Anteils enthält.

2. Verfahren nach Anspruch 1, worin die Wärme-Behandlung des in dem Lösungsmittel löslichen Anteils in der zweiten Stufe unter der folgenden Bedingung durchgeführt wird, worin T (°C) die Temperatur der Wärme-Behandlung und 8 (min) die Zeit, während der der Anteil auf der angegebenen Temperature gehalten wird, bezeichnen.

## Revendications

1. Procédé pour la production d'un brai approprie pour la préparation de fibres de carbone ledit procedé comprenant les étapes consistant a

(i) chauffer dans un premier stade, un brai obtenu de l'industrie du charbon,
(ii) extraire le brai ayant été ainsi traité à chaud avec un solvant,
(iii) séparer et éliminer la fraction insoluble dans le solvant conjointement avec le carbone libre et (iv) chauffer, dans un second stade, la fraction soluble dans la solvant, caractérisé en ce que
(v) le brai obtenu de l'industrie du charbon est un brai de houille grasse ou moyenne ayant un point de ramolissement deb 50 à 75°C,
(vi) le brai de houille est chauffe, dans le premier stade, a une temperature de 350 à 500°C sous atmosphère de gaz inerte, pour former une mésophase,
(vii) le solvant est un solvant aromatique,
(viii) la fraction insoluble dans le solvant contient la mésophase, et
(ix) la fraction soluble dans le solvant ne contient pas de carbone libre et elle est chauffée, dans le second stade, sous atmosphère de gaz inerte sous la pression atmosphérique ou sous pression réduite, pour former un brai en mésophase en masse, contenant 20-60% en poids de fraction insoluble dans la quinoléne.

2. Procédé selon la revendication 1, dans lequel le traitement thermique de la fraction soluble dans le solvant dans le second stade est effectué dans les conditions suivantes où T (°C) est la température du traitementtheremique et 8 (min) est la durée pendant laquelle ladite fraction est maintenue à cette température.
